

## UNITED STATES PATENT OFFICE

2,074,954

## METHOD OF TREATING METALS

Harvey Ross Belding, Vandergrift, Pa., assignor  
to American Sheet and Tin Plate Company, a  
corporation of New Jersey

No Drawing. Application June 17, 1935, Serial  
No. 27,088

## 2 Claims. (CL. 75—58)

This invention relates to a method of treating metals, and more particularly those which serve as a base for the application of vitreous enamel coatings.

5 In the manufacture of enamel ware, it has for some time been the practice to form, or draw, sheet steel and thereafter apply a vitreous enamel coating thereto. The coating is fused, or sintered, onto the base metal by the application of heat in 10 any suitable manner, but numerous difficulties frequently arise at this stage of the process. One of these difficulties is the formation during the fusing operation of objectionable defects in the surface of the enamel which is known as "reboiling" and is brought about by the condition of the base metal. These "reboiling" difficulties are due to bubbles of gas which are released from the base metal by the heating operation, and obviously mar the desired surface condition of the finished 15 enamel article.

20 It also very frequently happens that this gas released from the surface of the base metal by the heating operation causes an opening in the surface of the enamel to form other defects which are known in the art as "copper heads" or "fish scaling". These defects in the art of applying vitreous enamel coatings are not consistent, as they vary with the condition of the coating material and its time and temperature for fusing, 25 which, of course, change throughout the various fabricating plants.

It is among the objects of the present invention to provide a novel method of treating metals which are intended for the subsequent application 30 of vitreous enamel coatings in which there is a complete absence of "reboiling" or any tendency toward it.

Another object is the provision of a method of 35 the class described which will eliminate the "sensitivity of practice" in various fabricating plants notwithstanding minor variations in the condition of the coating material, firing time, and temperatures, which frequently give rise to the appearance of the defects previously discussed.

40 Another object is the provision of a novel method of the class described which may be easily and cheaply practiced with existing types of equipment to obtain very good results.

45 In its broadest sense the method provides for 50 the complete deoxidation or "killing" of the metal while in a molten state and within a time interval which minimizes the inclusion therein of gases.

The proposition of "killing" the molten metal 55 is, of course, very old in the art and generally

carried out by the addition to the ladle of aluminum, ferro-silicon or other deoxidizers, as the molten metal is being tapped from the melting furnace thereinto.

I have found that the addition of aluminum to the mold, or even the ladle, will not prevent "reboiling" when the metal is provided with vitreous enamel coatings, contrary to expectation.

The method of the invention distinguishes over 10 the prior art in that the molten metal is "killed" by the sole addition to the mold, and during the "teeming" of the molten metal thereinto from the ladle, of silicon only, in the form of ferro-silicon or refined silicon.

15 It is well known in the art that aluminum is a more powerful and complete "killing" agent than silicon, but I have found that the addition of silicon-and-aluminum either to the ladle or mold will not produce a metal having "non-reboiling" 20 characteristics. This is true regardless of the sequence of adding silicon-and-aluminum, whether mixed or otherwise.

25 Metals of the type described (intended for the subsequent application of vitreous enamel coatings) are usually of the "low metalloid" variety and contain less than 0.10 per cent carbon and 0.50 per cent manganese. In practicing my invention I may produce steel for subsequent enameling which has a carbon content of approximately 0.025 per cent and a manganese content of 30 approximately 0.08 per cent. This steel is then poured in its molten condition from a refining furnace into a ladle, which is identified in the art as the "tapping" operation. As the molten steel is being "teemed" from the ladle into the mold, silicon (in the form of ferro-silicon or refined silicon) is added to the mold, resulting in 35 the rapid and effective "killing" of the steel at this point of its manufacture.

40 As a specific instance, a very satisfactory result has been obtained by adding approximately two pounds of 90 per cent ferro-silicon to the mold for each net ton of steel being treated, and while the latter is being "teemed". The addition of the ferro-silicon to the mold may be gradual (whether intermittent or otherwise), if desired. It is to be understood that the amount of silicon added in the manner previously described may be 45 reduced somewhat if the steel is higher in carbon or manganese. Also, for instance, if the ferro-silicon contains less than 90 per cent available silicon its ratio must be increased. I have found 50 that the more expensive alloy of higher silicon 55

content is much to be preferred, as the "killing" action is more rapid and pronounced.

After the steel has been completely "killed" it is subsequently processed to desired form or shape 5 according to any of the well known practices.

If, by way of example, enameled sheets are intended as the final article, the uncoated sheets are subjected to the usual coating of vitreous enamel which is fused thereon by firing or heating in a 10 suitable furnace to a temperature of from 1550 degrees Fahrenheit to 1625 degrees Fahrenheit, and then permitted to cool to room temperature. After the coating of vitreous enamel has cooled, at least one final covering coat of vitreous enamel 15 is usually applied thereto. If this covering coat is applied, the sheet is again fired or heated to burn it on the metal. It is during this firing or heating that the metal "reboils" and develops gas "bubbles" or the "copper-heads" or "fish scales" 20 previously mentioned. Due to the treatment of the molten metal in accordance with the teaching of the present invention, a vitreous enameled article is obtained having a perfectly smooth and uninterrupted surface condition.

25 The preferred method of rolling strip metal is usually in the direction of the axis of the original ingot, and if this is followed, the metal resulting from the foregoing treatment will consistently produce excellent results. If, on the other hand, 30 the equipment of the mill is such as to necessitate the rolling of the strip in a direction which is transverse to the axis of the original ingot, the metal produced by the method of the invention 35 has a somewhat increased tendency toward a seamy surface.

While these resultant seams are in no way connected with "reboiling" characteristics, they nevertheless are sometimes objectionable from the 40 standpoint of appearance after enameling. If it

is necessary to process the metal in this manner, and seams result, I have found that they may be expeditiously removed by bombarding an abrasive upon them. This abrasive (as, for example, grit) removes the seams to such an extent that they are 5 no longer objectionable. This bombardment with an abrasive is an inexpensive operation (as it, of course, obviates the necessity of the usual pickling operation), and may be of short duration, as the 10 seams, if any, will be very shallow.

Iron or steel made after the manner of my invention will usually contain from 0.015 to 0.10 per cent silicon, but it is the presence in the iron or 15 steel of silicon in approximately such amounts, which silicon has been added to the steel in the particular manner I have described, that produces the improvement which I claim for my process, rather than the mere presence of silicon as such 20 in the iron or steel, without reference to the manner of addition.

While I have shown and described one specific embodiment of my invention, it will be understood that I do not wish to be limited exactly thereto, since various modifications may be made without 25 departing from the scope of my invention, as defined in the following claims.

I claim:

1. The method which includes teeming molten 30 steel into a mold, killing the molten steel while in the mold solely by the use of silicon, forming the killed steel into articles, and coating the articles with vitreous enamel.

2. The method which comprises teeming molten 35 steel into a mold, killing the molten steel during the teeming step solely by the use of silicon, forming the killed steel into articles, and coating the articles with vitreous enamel.

HARVEY ROSS BELDING.